

## UNITED STATES PATENT OFFICE

ERNST BECKER, OF HAMBURG, GERMANY, ASSIGNOR TO I. G. FARBENINDUSTRIE AKTIENGESELLSCHAFT, OF FRANKFORT-ON-THE-MAIN, GERMANY, A CORPORATION OF GERMANY

## PROCESS OF PREPARING VULCANIZED FIBERS

No Drawing. Application filed May 29, 1929, Serial No. 367,135, and in Germany June 4, 1928.

The present invention relates to the manufacture of vulcanized fibers and the like by means of sulfuric acid according to the roller or continuous process.

5 The manufacture of vulcanized fibers and the like by means of sulfuric acid is technically very difficult since the sulfuric acid soon destroys the paper used.

In accordance with the present invention 10 the action of the sulfuric acid on the paper is completely regulated and retarded by the addition of a soluble salt which is not decomposed by the sulfuric acid, for example, alkali metal sulfates, ammonium sulfate, and 15 magnesium sulfate. These salts counteract the dispersing action of the sulfuric acid; the solution of the paper proceeds much more slowly, which enables the paper to be rolled into a fiber plate on the rollers. The action 20 of the soluble salts, such as for example sulfates, increases with the valency of the base, apart from the quantity added. It is of particular value that the hydration or parchmentizing of the cellulose can in this manner 25 be varied to a far reaching extent, that is to say vulcanized fibers and the like of homogeneous character and high specific gravity and likewise more fibrous, flexible fiber of low specific gravity can be manufactured as 30 desired.

Furthermore, for the manufacture of vulcanized fibers, parchment paper and the like by the continuous process on the so-called parchmentizing machine an acid with the additions specified can be used with advantage, especially when it is desired to weaken the action of the sulfuric acid, for example, in the case of certain wood pulp papers and the like.

40 The invention is illustrated by some of the compositions of the baths in question, but is not limited thereto:

Example 1.—The parchmentizing bath contains: 68% sulfuric acid 1/2-2% magnesium sulfate.

Example 2.—The parchmentizing bath contains: 70% sulfuric acid 4-5% ammonium sulfate.

I claim:

1. In the process for the manufacture of

vulcanized fibers and the like, the step which comprises parchmentizing paper with sulfuric acid to which a sulfate soluble in sulfuric acid has been added.

2. In the process for the manufacture of 55 vulcanized fibers and the like the step which comprises parchmentizing paper with sulfuric acid to which 0.5 to 5% of a sulfate soluble in sulfuric acid has been added.

3. In the process for the manufacture of 60 vulcanized fibers and the like the step which comprises parchmentizing paper with sulfuric acid to which ammonium sulfate has been added.

4. In the process for the manufacture of 65 vulcanized fibers and the like the step which comprises parchmentizing paper with sulfuric acid to which 4 to 5% of ammonium sulfate has been added.

In testimony whereof I have hereunto set 70 my hand.

ERNST BECKER.